

Oct. 8, 1929.

W. F. HARVEY

1,731,099

METHOD OF FORMING A CEMENT RECEIVING SURFACE ON AN INSULATOR SECTION

Filed May 3, 1926

Fig. 1



Fig. 2



Fig. 3



Fig. 5



Fig. 6



Fig. 4



INVENTOR

William F. Harvey  
Harold E. Stonebraker  
BY  
his ATTORNEY

## UNITED STATES PATENT OFFICE

WILLIAM F. HARVEY, OF LIMA, NEW YORK; MARY J. HARVEY EXECUTRIX OF SAID  
WILLIAM F. HARVEY, DECEASED

## METHOD OF FORMING A CEMENT-RECEIVING SURFACE ON AN INSULATOR SECTION

Application filed May 3, 1928. Serial No. 106,382.

My invention relates to a method of forming a cement receiving surface on one of the sections of an insulator, having reference more particularly to providing a porcelain 5 insulator section of a multipart insulator with an integral surface of such character as to form a tight bond with the cement between the sections, although the surface obtained and the method employed are applicable to other 10 uses as well.

The usual practice heretofore in cementing insulator sections has been to provide one of the sections with a cement receiving surface of sand or crushed particles which are affixed 15 to the porcelain body by a glaze or other securing medium, and it is a purpose of my invention to eliminate the necessity of securing sand or like particles to the porcelain body, and to afford a closer bond between the 20 cement and porcelain by a method requiring less time, and which is cheaper to employ than where sand or crushed particles are secured to the porcelain body.

In a more particular aspect, the invention 25 has for its object to provide a porcelain insulator section with an irregularly roughened surface formed by indenting the porcelain while wet, in a manner to exactly simulate a surface composed of sand or like particles, thereby obtaining a cement receiving 30 surface directly on the surface of the porcelain and having the same contour and exterior characteristics of a sanded surface.

The invention consists further in producing 35 the desired roughened surface on the porcelain body by means of a tool or die-member which may have its operative surface composed of sand or crushed particles, or may have an operative surface formed by indenting 40 the die-member with a master die of sand or crushed particles, so that it is possible to obtain on the porcelain surface of the insulator section a cement receiving surface which is either an exact duplicate of a surface composed of sand or like particles, or is substantially complementary to such a sanded surface.

Still a further purpose of the invention is 45 to provide a method and means by which a porcelain insulator section can be roughened or indented in less time and at less cost than

where a sanded surface is employed, obtaining a surface that has all the advantages of a sanded surface and possesses certain points of superiority thereover.

With these and other ends in view, the invention consists in the structure and procedure that will appear from the following description when read in conjunction with the accompanying drawing, the novel characteristics being pointed out in the claims following the description.

In the drawing:

Figure 1 is a sectional view of one type of insulator made in accordance with the invention;

Figure 2 is a side elevation of the inner section of the insulator, showing the relative position of the tool or die-member in applying the cement receiving surface to the insulator section;

Figure 3 is a side elevation of the tool;

Figure 4 is a sectional view of a modified form of tool;

Figure 5 is an enlarged sectional view of a portion of an insulator section, showing the indentations forming the cement receiving surface when made by a positive die member, and

Figure 6 is a similar view showing a cement receiving surface when produced by a negative die-member.

The invention is applicable to various products where a roughened surface is desirable, and may be practiced in many different ways other than what is set forth herein. This application is not intended to limit the invention in construction, form of procedure, or adaptation, but is merely to set forth a practical embodiment that is exemplary of its practical field of use.

Figure 1 illustrates a known type of two-part insulator to which the invention can be applied, and which comprises an inner section 1 and an outer section 2, held together by a body of cement 3 between them.

The general procedure in cementing this type of insulator heretofore has been to provide on the inner section 1 a cement receiving surface of sand or crushed particles that are attached to the surface of the porcelain

body by means of a glaze or the like, such sanded surface being affixed to the porcelain body before the cement is inserted between the sections. According to my invention, no sand or crushed particles need be secured to the surface of the porcelain body, and the same effect is obtained by providing the cement receiving surface of the porcelain body with an irregularly roughened or indented area that simulates and has the same exterior characteristics as a sanded surface.

This result is accomplished by using a tool or die-member, as illustrated at 4, and applying it to the desired surface of the porcelain section while the latter is in a wet state, and before baking. The tool or die-member may comprise a cylindrical roller as shown, mounted on a suitable handle 5, so that it can readily be held in operative relationship to the porcelain, preferably by mounting the insulator section on a suitable support that is rotated while the tool is maintained against the surface. Or the tool may take the form of a ring, band or stamping device, or other character adapted for reproducing its operative surface on the porcelain body.

The tool or die-member 4, as shown in Figures 2 and 3, includes a body portion to the periphery of which are attached a multiplicity of sand or crushed particles, by gluing or otherwise, to afford an irregular, sand-like surface that is pressed against the porcelain body of the insulator. Where a sanded surface is used on the tool or die-member, as shown in Figure 2, the irregularly roughened or indented cement receiving surface on the insulator section is complementary to the sand or crushed particles on the die-member.

In order to reduce the cost of operation, the cylindrical portion of the tool or die-member may be made of porcelain, as shown in Figure 4, in which case its operative surface 6 is formed, while the porcelain is wet, by rolling thereagainst a master die having an operative surface composed of sand or crushed particles. Thus one master die can be used to make a large number of porcelain tools such as shown in Figure 4. When thus formed, the surface 6 on the tool is complementary to the master surface of sand or crushed particles. When this complementary or negative tool or die-member, illustrated in Figure 4, is rotated against the porcelain body of the insulator section, the indentations or roughened surface formed thereon becomes positive, and is a substantial duplicate of the surface composed of sand or crushed particles.

Figure 5 illustrates a cement receiving surface on the insulator section made by a positive tool or die-member, as where sand or crushed particles constitute the operative surface of the tool, the indented surface being negative, or complementary to the positive tool, whereas Figure 6 shows a cement receiving surface that is positive, or complementary to

a negative tool, such as illustrated in Figure 4. In either case, the surface produced forms a perfect bond or union with the cement that is more efficient and will stand greater strains than where sand or crushed particles are attached to the porcelain insulator section to obtain a roughened surface. The carrying out of the invention described involves a substantial reduction in cost because the required tools can be made cheaply, and it requires only a second or two to bring the tool and insulator section into operative relation and completely indent the surface in the porcelain.

The tool or die-member and the method of procedure described may be modified, and this application is intended to cover any changes or departures that accomplish the same result and come within the intent of the invention or the scope of the following claims.

I claim:

1. The method of forming a cement receiving surface on an insulator section which consists of roughening the porcelain surface irregularly while wet.

2. The method of forming a cement receiving surface on an insulator section which consists in subjecting the porcelain surface while wet to the indenting action of a multiplicity of sand-like particles.

3. The method of forming a cement receiving surface on an insulator section which consists in subjecting the porcelain surface while wet to the indenting action of an irregular surface having the characteristics of sand-like particles.

In witness whereof, I have hereunto signed my name.

WILLIAM F. HARVEY.

105

110

115

120

125

130